

## UNITED STATES PATENT OFFICE

2,318,322

METHOD FOR PRODUCING LACQUER OR  
VARNISH RESIST

Charles Edmund Meulendyke, Rochester, N. Y.

No Drawing. Application August 7, 1940,  
Serial No. 351,783

6 Claims. (Cl. 41—43)

This invention relates to the preparation of photomechanical printing plates as generally adapted to relief, planographic, and intaglio printing in either monochrome or polychrome.

Reference is made to co-pending patent application of C. E. Meulendyke, filed June 7, 1939, Serial No. 277,843. In this invention, a metallic support such as a copper plate electroplated with a nickel layer directly supports a lacquer or varnish layer, which in turn supports a colloid layer containing a sensitive silver salt. The emulsion layer after being exposed under a suitable half-tone or line negative is developed and processed into a colloid relief with bared lacquer or varnish areas. The lacquer or varnish layer is then cut through to form a lacquer or varnish relief under the selective control of the emulsion resist, and the bared metallic areas are then etched in an appropriate solution to form a relief printing plate. Primarily, this invention is concerned with the step of cutting through the lacquer or varnish layer. It is not concerned with whatever subsequent appropriate etching method may be used for final conversion of such system into a metallic printing plate.

In a system consisting of a metallic layer supporting a lacquer or varnish layer, which in turn supports suitable local resists, it has been generally suggested to cut through the lacquer or varnish layer in a simple solvent appropriate to the lacquer or varnish. Thus cellulose nitrate or cellulose acetate can be cut through with acetone, gum shellac with alcohol, or bitumen with benzol. It has been suggested that such cutting can be aided by gentle rubbing with a pad of cotton wool moistened with the solvent, or by brushing with a camel's hair brush.

In the etching of metal, there is a clean-cutting action at the surface of the metal. In cutting through a lacquer or varnish layer, however, we are dealing with colloid phenomena and with conditions of swelling and gel formation which complicate the removal of the lacquer or varnish. In the use of an ordinary varnish remover, it is recommended to first swell the varnish, then to scrape off the gel formation. For such purposes as in this invention, however, the operation of forming a secondary lacquer resist with clean-cut half-tone dots and clean bared metallic areas in accurate conformity to the dots of the primary resist, presents a delicate operation which cannot be satisfactorily performed by use of the solvent action of the appropriate solvent alone. Excessive swelling and absorption of the solvent and creeping of

the absorbed solvent along the interface of the primary resist can cause loosening of the bonding between the varnish layer and the primary resist, and especially can cause undercutting of such primary resist before the solvent action has cut the varnish through to form bared metallic areas for subsequent etching.

I have found that the cutting through of the lacquer or varnish layer in such a system as described above can be accomplished without the troublesome colloid phenomena of swelling and gel formation. In other words, I have found that such operation can be carried out under conditions substantially analogous to the etching of metal, such as the etching of copper with ferric chloride. For example, let us take the case of a layer of gum shellac. The appropriate solvent of gum shellac is ethyl alcohol. Gum shellac is readily soluble in ethyl alcohol with the usual concomitants of swelling, diffusion, and gel formation, which for my purposes I wish to avoid. I have found that if I add an equal volume of glycerine to the alcohol, its solvent action upon the gum shellac layer becomes practically nil. I now take advantage of the fact that gum shellac and resins in general are destroyed in the presence of strong alkalis, that resins in general are soluble in alcohol, and that alcohols in general can dissolve considerable quantities of strong alkalis such as potassium, sodium and lithium hydroxides.

I have found that a solution of equal quantities of ethyl alcohol and glycerine has practically no solvent action on gum shellac but that this same solution saturated with a strong alkali will cut through the shellac in a manner analogous to the etching of metal, that is to say, the cutting action takes place in situ at the exposed surface of the shellac where it comes into contact with the cutting medium. The alcohol and glycerine may be said to function as the vehicle for bringing the caustic alkali as the active cutting agent into contact with the shellac. The alcohol used is preferably the 95% grain or denatured alcohol of commerce. Water in any appreciable amount can cause loosening of the primary local resists, usually of gelatin, from the lacquer or varnish layer and its presence should be avoided. For the same reason care should be taken that the glycerine used is water-free. Gelatin itself is totally impermeable to water-free alcohol or water-free glycerine or to mixtures of the same in any proportion. However, after the desired cutting action on the resinous layer has been attained, the system

may be flushed with water to remove residual solvent mixture and any thin film of water-soluble resinate which may have formed.

Within the meaning of this invention, I mean to include in the resinous layer any suitable natural gums or resins such as shellac, copal, dammar, dragon's blood, etc., as well as artificial resins. Also I intend to include alcohol-soluble cellulosic derivatives such as cellulose nitrate, cellulose acetate, etc., used in conjunction with resinous substances. Within the meaning of the term "alcohol," I mean to include those alcohols or equivalents solvents capable of dissolving sufficient alkali to carry out the operations substantially as herein described. While I suggest glycerine as especially useful to function in increasing the viscosity of the solution and in restraining the solvent action of alcohol, I intend to include any suitable ingredient capable of functioning in an analogous manner.

As a correlated part of this invention, I have further found that the cutting through of the lacquer or varnish layer in such a system as described above is facilitated by adding to the appropriate solvent an ingredient which is an etchant of the metallic surface. As a specific example, we may take the system of a nickel layer supporting a gum shellac layer which in turn supports suitable local resists. Cupric chloride and ferric chloride which readily etch nickel are easily soluble in alcohol. The cupric chloride and ferric chloride, besides serving as etchants of the metallic surface, increase the viscosity of the solution and act as restrainers on the solvent action of the alcohol and as inhibitors to prevent the troublesome colloid phenomena of diffusion, swelling, and gel formation. This etching action at the metallic surface is a superficial one and is very effective in breaking up and removing last traces of resin in areas to be bared and in producing a clean-cut resinous resist for the subsequent etching of the metal.

It will thus be seen that I have described processes with all necessary details embodying the principles and attaining the objects and advantages of the invention. Since many matters of treatment, manipulation, selection, and proportion of ingredients, succession of steps, and other details may be variously modified without departing from the principles involved, I do not intend any limitation to such details excepting so far as set forth in the appended claims.

What is claimed is:

1. The method of producing resinous reliefs or resinous resists by cutting into or through a suitably supported resinous layer supporting suitable local resists with an alcoholic solution made strongly alkaline and including an ingredient to increase the viscosity of such solution and to re-

strain the solvent action of the alcohol, such ingredient being present in such proportion that the solvent mixture without presence of the alkali has no appreciable solvent action on the resinous layer but serves rather as vehicle to bring the alkali into contact with the resin, thus avoiding troublesome colloid phenomena substantially as herein described.

2. The method of producing resinous reliefs or resinous resists by cutting into or through a suitably supported resinous layer supporting suitable local resists with an alcoholic solution made strongly alkaline with caustic alkali and including glycerine to increase the viscosity of such solution and to restrain the solvent action of the alcohol, the glycerine being present in such proportion that the solvent mixture without presence of the alkali has no appreciable solvent action on the resinous layer but serves rather as vehicle to bring the alkali into contact with the resin, thus avoiding troublesome colloid phenomena substantially as herein described.

3. The method of producing resinous reliefs or resinous resists by cutting into or through a suitably supported resinous layer supporting suitable local resists with an alcoholic solution saturated with caustic alkali and containing an equal volume of glycerine, substantially as herein described.

4. The method of producing resinous resists by cutting through a resinous layer supported on a suitable metallic layer and supporting suitable local resists with an alcoholic solution including an ingredient which restrains the solvent action of the alcohol and an ingredient which superficially etches the metallic surface, thereby loosening and removing last traces of resin in the metallic areas desired to be bared for subsequent etching, substantially as herein described.

5. The method of producing resinous resists by cutting through a resinous layer supported on a suitable metallic layer and supporting suitable local resists with an alcoholic solution including cupric chloride as an ingredient to restrain the solvent action of the alcohol and to superficially etch the metallic surface thereby loosening and removing last traces of resin in the metallic areas desired to be bared for subsequent etching, substantially as herein described.

6. The method of producing resinous resists by cutting through a resinous layer supported on a suitable metallic layer and supporting suitable local resists with an alcoholic solution including ferric chloride as an ingredient to restrain the solvent action of the alcohol and to superficially etch the metallic surface thereby loosening and removing last traces of resin in the metallic areas desired to be bared for subsequent etching, substantially as herein described.

CHARLES EDMUND MEULENDYKE.